

# UNITED STATES PATENT OFFICE.

THOMAS A. JENCKES, OF PROVIDENCE, RHODE ISLAND.

## IMPROVED WATER-PROOF FABRIC.

Specification forming part of Letters Patent No. 34,428, dated February 18, 1862.

*Whom it may concern:*

Be it known that I, THOMAS A. JENCKES, of the city and county of Providence, and State of Rhode Island, have invented a new Napped Water-Proof Fabric composed of india-rubber or allied gums, in combination with textile fabrics and with flocks or fibers of wool, fine silk, and other fibrous substances, and which constitutes a new manufacture; and I do hereby declare that the following is a full and exact description thereof.

The base of the new fabric is cloth or any textile fabric finished evenly and smoothly. This is made to pass between revolving metallic rolls so gaged as to leave an opening of about the thickness of the fabric. The india-rubber or other gum is prepared in any of the ordinary modes, by grinding, or by dissolving, or (which I have found the best) by being partially dissolved and then softened to the proper uniform consistency for working by grinding. The prepared rubber or other gum is fed between the rolls and upon the cloth or other fabric, or is otherwise spread thereon before entering the rolls in any of the known modes. The pressure of the rolls should be so great as to incorporate the rubber or other gum thoroughly with the fabric, and not merely cover it or coat it. A surface of gum will be left upon one side of the fabric, and upon this is sifted or spread by hand or by machinery a coating of flocks of wool, fur, silk, or other fibrous substances or disintegrated fiber, in such manner that each fiber shall fall as nearly as possible by itself without being attached to or felted with any other fibers. This result may be obtained in a very satisfactory manner by the use of a machine patented to John F. Green on the 26th day of February, A. D. 1861. The fabric thus spread or covered with flock or fiber is again made to pass between the rolls at a great pressure, and the flock or fiber is pressed into the rubber and the textile fabric with which it has become combined, so that the cloth, rubber, or other gum and the flock or fiber are pressed together and form integral portions of the new compound fabric. If one operation is not sufficient, it should be repeated till the result is attained. Any surplus flock or fiber that may have fallen upon the fabric and not have become incorporated with it should be brushed off, and by the same operation of brushing a nap may be raised of

the flock or fiber which has become a part of the fabric, or the nap may be raised by processes well known in the treatment of cloths. The nap may also be sheared and rendered as even as that of broadcloth. When flocks or fibers of fur are used their length and softness have the effect of producing a peculiarly smooth, soft, and even surface; and the water-repellent properties of this article give it also a superior value. The fabric may be dyed, pressed, and finished like cloth.

It is obvious that rolls of a large size and great weights, when capable of nice adjustment, are preferable to those of a light and slender make, and that these rolls must have the apparatus for adjustment as to position and speed of revolution and for being heated and cooled well known among india-rubber manufacturers.

An improved result is also attained by vulcanizing the india-rubber or other vulcanizable gum in the new fabric.

In all previous manufactures of napped or flocked india-rubber fabrics, or those made with similar gums, the flock or fiber has been made to adhere to the fabric which forms the base by thin solutions of gum or by a cement made from it, and the pressure to which the combination has been subjected has been merely for the purpose of causing the gum to adhere to the surface of the cloth or other fabric and the flocks or fibers to adhere to the coating or surface of gum. In these former combinations the cloth or other fabric was liable to peel off or separate from the gum, and the flock or fiber would soon rub or wear away. Besides, the finished fabric would not be certainly water-proof. These and other defects which have prevented the flocked fabrics from coming into general use are completely obviated by my invention.

What I claim as my invention, and desire to secure by Letters Patent, is—

The fabric in which flocks or fibers and india-rubber or allied gums are combined with cloth or other base by means of pressure so as to become integral portions of the new napped water-proof fabric, substantially as described, the same being a new manufacture.

THOMAS A. JENCKES.

Witnesses:

H. W. PEICE,  
A. B. STOUGHTON.